

# United States Patent Office

3,166,410

Patented Jan. 19, 1963

1

3,166,410  
FORGING BRASS ALLOY CONTAINING SMALL  
AMOUNTS OF BERYLLIUM  
Philip S. Hanson, Wyoming, and Robert E. Saxtan,  
Reading, Pa., assignors to The Beryllium Corporation,  
Reading, Pa., a corporation of Delaware  
No Drawing. Filed Apr. 29, 1963, Ser. No. 276,155  
5 Claims. (Cl. 75—153)

This invention relates generally to improvements in 10 forging brass alloys.

A general object of the present invention is to provide a new forging brass alloy composition which can be hot forged, easily machined and hardened and in which the machining may be done in the hardened state.

Standard brass forgings are soft after forging, having Rockwell readings in the neighborhood of F75-80. Such standard forging brass having a Rockwell hardness of F-78 is not subject to thermal treatments for changes in hardness except to a very minor degree. Such standard forging brass is generally measured on the Rockwell F scale. Rockwell B readings are generally below Rockwell B-50.

The objectives of the present invention to improve the properties of forging brass are attained by the addition of a small percentage of beryllium to an alloy, comprising essentially copper, lead, and zinc.

The addition of a small percentage of beryllium to this composition produces an alloy which can be hot forged, easily machined and hardened and also an alloy which may be machined in the hardened state.

The present improved forging brass alloy has the following general or nominal composition:

58.0-68.0 percent copper  
1.5-2.5 percent lead  
.18-.7 percent beryllium  
Balance—Zinc

The solution heat treating temperature for this improved alloy is extremely fine grained, easily workable and capable of being hardened by solution heat treating, quenching and ageing.

The solution heat treating temperature for this improved alloy is in the range of from 1050° F. to 1500° F. The higher temperatures for the solution heat treating increase the percentage beta present and thus higher or greater hardness is obtained after ageing.

The preferred ageing temperature for the alloy is 600° F. for a period of approximately 3 hours. Temperatures lower than 600° F. may be used for a longer period of time and temperatures above 600° F. will accelerate the ageing and therefore a shorter time can be used.

The preferred composition has a beryllium content within the range of from .25 to .4 percent.

A percentage lower than .18 percent of beryllium in the alloy will bring about a slight increase in hardness due to solid solution hardening but the response to ageing treatments is somewhat less than that obtained when the beryllium content is above .18 percent and within the range set forth above.

The following tabulations set forth the different properties for the alloy having the beryllium content within the stated nominal composition range and as distinguished between solution annealed and quenched material and materials subject to solution annealing, quenching and ageing, employing the solution heat treating temperatures in the range hereinabove set forth and the ageing temperature stated.

In the alloy composition having a beryllium content

2

in the area of .2 percent, a Rockwell B hardness increase of from 3 to 5 points will be shown between the solution annealed and quenched materials and solution anneal, quench, and age as follows:

.2% Be typical properties:

Solution anneal—Rockwell B-60-68

Solution anneal and age—Rockwell B68-72

Where the beryllium content of the alloy is on the high side as, for example, approximately .6 percent in the composition, a considerable increase in solid solution hardening plus age hardening response is shown in accordance with the following set forth properties:

.6% Be typical properties:

Solution anneal—Rockwell B70-80

Solution anneal and age—Rockwell B92-100

The Rockwell range is a function of the solution anneal temperature. The low range represents lower temperatures which display lower beta percentages and greater ductility. The higher Rockwell readings mean higher beta percentages and less ductility.

For the preferred beryllium range in the composition, namely, the mid range values of from .25 to .4 percent beryllium, the typical properties are as follows:

Solution anneal—Rockwell B60-80

Solution anneal and age—Rockwell B82-95

The preferred beryllium range also gives the best combination of ductility and hardness.

Additional features of the beryllium additions are evident, viz.: the alloy can be air cooled with lower resulting hardnesses and lessened response to ageing but with some response and especially so in the higher beryllium ranges.

The composition when containing the beryllium in the range of from .4 to .5 percent has the following properties or characteristics when annealed at the indicated temperatures and quenched and when aged at the temperature indicated, following the annealing and quenching.

Anneal 1275° F. and quench—Rockwell B60-70

Age 600° F. for 3 hours—Rockwell B85-90

Anneal at 1275° F. and air cool—Rockwell B50-60

Age 600° F. for 3 hours—Rockwell B70-80

A specific example of the forging brass alloy of the present invention is given as follows:

|           | Percent |
|-----------|---------|
| Copper    | 63.07   |
| Lead      | 2.5     |
| Beryllium | .50     |
| Balance   | Zinc    |

The foregoing alloy composition was annealed at 1250° F. for 30 minutes and water quenched. This sample of the alloy showed the Rockwell B hardness of 80-85.

Ageing the sample having the above composition for 3 hours at 600° F. showed a Rockwell B hardness of 85-96.

Samples of the beryllium brass were prepared and thermally treated and tested for mechanical properties.

The following table sets forth the chemical composition of three such samples having the identification markings set forth:

| Identification | Cu, Percent | Be, Percent | Pb, Percent | Zn   |
|----------------|-------------|-------------|-------------|------|
| Strip A        | 68          | 0.5         | 0.5         | Bal. |
| Rod B          | 68          | 0.5         | 0.5         | Bal. |
| Rod C          | 63          | 0.5         | 2.5         | Bal. |

Mechanical properties are as follows:

Table I—Beryllium brass strip

| Processing                                         |   | U.T.S.,<br>p.s.i. | Y.S.,<br>0.2%,<br>p.s.i. | 0.5%<br>Total<br>Strain<br>under<br>Load,<br>p.s.i. | Elong.,<br>Percent | Rock-<br>well<br>B |
|----------------------------------------------------|---|-------------------|--------------------------|-----------------------------------------------------|--------------------|--------------------|
| 1. Cold rolled from .180 to .100                   | A | 106,000           | 88,300                   | 65,400                                              | 3                  | 96                 |
| 2. Same as #1 plus 2 hours at 600° F.              | A | 98,300            | 84,800                   | 64,300                                              | 10                 | 96                 |
| 3. S.H.T. $\frac{1}{2}$ hour at 1250° F., W.Q.     | A | 68,600            | 29,300                   | 31,500                                              | 43                 | 65                 |
| 4. Same as #3 plus 3 hours at 600° F.              | A | 85,500            | 55,800                   | 49,200                                              | 30                 | 86                 |
| 5. S.H.T. $\frac{1}{2}$ hr. at 1250° F., Air Cool. | A | 68,600            | 33,800                   | 34,500                                              | 37                 | 68                 |
| 6. Same as #5 plus 3 hours at 600° F.              | A | 75,400            | 43,400                   | 43,400                                              | 30                 | 78                 |

Table II—Beryllium brass rod

| Processing                                         |   | U.T.S.,<br>p.s.i. | Y.S.,<br>0.2%,<br>p.s.i. | 0.5%<br>Total<br>Strain<br>under<br>Load,<br>p.s.i. | Elong.,<br>Percent | Rock-<br>well<br>B |
|----------------------------------------------------|---|-------------------|--------------------------|-----------------------------------------------------|--------------------|--------------------|
| 1B. Cold drawn from 1.0" dia. to .780" dia.        | B | 105,100           | 86,100                   | 57,100                                              | 6                  | 93                 |
| 2. Same as #1B plus 2 hrs. at 600° F.              | B | 111,500           | 102,900                  | 75,500                                              | 7                  | 99                 |
| 3. S.H.T. $\frac{1}{2}$ hr. at 1250° F., W.Q.      | C | 96,700            | 86,700                   | 56,500                                              | 8                  | 95                 |
| 4. Same as #3 plus 3 hrs. at 600° F.               | B | 70,600            | 35,900                   | 35,900                                              | 38                 | 69                 |
| 5. S.H.T. $\frac{1}{2}$ hr. at 1250° F., Air Cool. | C | 86,400            | 41,600                   | 25,500                                              | 20                 | 81                 |
| 6. Same as #5 plus 3 hrs. at 600° F.               | B | 93,400            | 65,900                   | 64,900                                              | 26                 | 88                 |
|                                                    | C | 100,500           | 67,000                   | 47,100                                              | 13                 | 90                 |
|                                                    | B | 71,200            | 37,200                   | 37,200                                              | 35                 | 70                 |
|                                                    | C | 68,600            | 28,500                   | 17,500                                              | 23                 | 74                 |
|                                                    | B | 77,800            | 40,000                   | 40,000                                              | 29                 | 76                 |
|                                                    | C | 79,100            | 42,300                   | 34,400                                              | 23                 | 78                 |

The above set forth results of the tests made on the forging brass alloy containing beryllium in the amount of .5 percent, as set forth clearly illustrate the improvements obtained over standard forging brass not having beryllium alloyed therein.

We claim:

1. A forging brass alloy consisting of the following constituents in the following range proportion:

|           | Percent      |
|-----------|--------------|
| Copper    | 58.0 to 68.0 |
| Lead      | 1.5 to 2.5   |
| Beryllium | 0.18 to 0.70 |
| Balance   | Zinc         |

2. A forging brass alloy consisting of:

|           | Percent |
|-----------|---------|
| Copper    | 63.07   |
| Lead      | 2.5     |
| Beryllium | .50     |
| Balance   | Zinc    |

3. A forging brass consisting of:

|           | Percent |
|-----------|---------|
| Copper    | 63.07   |
| Lead      | 2.5     |
| Beryllium | .50     |
| Balance   | Zinc    |

and having a Rockwell hardness of B85-96.

4. A forging brass alloy consisting of 58 percent to 68 percent copper, 1.5 percent to 2.5 percent lead, 0.18 percent to 0.70 percent beryllium, and the balance zinc, having a high beta content, a Rockwell B hardness of 90-97, and being fine grain.

5. A forging brass consisting of:

|           | Percent      |
|-----------|--------------|
| Copper    | 58.0 to 68.0 |
| Lead      | 1.5 to 2.5   |
| Beryllium | 0.18 to 0.70 |
| Balance   | Zinc         |

and having fine grain, high beta content, and capable of being hardened by solution heat treating, quenching and aging.

References Cited in the file of this patent

UNITED STATES PATENTS

|           |                 |                |
|-----------|-----------------|----------------|
| 1,880,223 | Weymouth et al. | Oct. 4, 1932   |
| 2,296,706 | Corson          | Sept. 22, 1942 |
| 2,311,750 | Hensel et al.   | Feb. 23, 1943  |